

Aug. 9, 1932.

P. C. WAITE

1,871,249

RUG AND METHOD OF MANUFACTURING THE SAME

Filed March 1, 1930

Fig. 1.



Fig. 2.



Fig. 3.



Fig. 4.



Inventor

Philip C. Waite

By Samuel W. Banning  
J. H. G.

## UNITED STATES PATENT OFFICE

PHILIP C. WAITE, OF OSHKOSH, WISCONSIN, ASSIGNOR TO WAITE CARPET COMPANY,  
OF OSHKOSH, WISCONSIN, A CORPORATION OF WISCONSIN

## RUG AND METHOD OF MANUFACTURING THE SAME

Application filed March 1, 1930. Serial No. 432,455.

This invention relates to rugs and method of manufacturing the same.

The present invention is directed to a method of making, dyeing and finishing rugs tufted with rayon silk, and has for its object to produce a pile surfaced rug having a fur-like texture adapted to reflect the light in such a way as to present a beautiful sheen, and in which the fine rayon fibres or filaments

10 are so intermeshed and intermingled as to conceal the presence of the separated tufts composing the pile of the rug.

In the manufacture of rugs in accordance with the method of the present invention, I employ a ground or backing which is preferably of canvas or similar fabric, and stitch the backing material with rows of stitches, which are in each instance looped and cut on the front side of the rug to form closely spaced rows of separated tufts, which stand 20 away from the backing and constitute the pile of the present invention.

A suitable method and mechanism for forming the tufts constitutes the subject matter of co-pending application, Serial No. 25 428,872, filed February 17, 1930, so that it is not here deemed necessary to describe said method or mechanism in detail.

In order to secure the sheen effect, which 30 is the characteristic feature of the present invention, I employ in the tufting and stitching, bundled strands of rayon filaments known in the trade as thrown rayon strands, in which the individual filaments are of exceeding fineness and possess a luster which 35 peculiarly adapts them to the requirements of the present invention.

The bundled strands of thrown rayon are 40 only slightly twisted to maintain the strands in bundled formation, so that when the tufts have been formed, the individual rayon filaments will easily spread out or separate from one another to present their tips in diverging relation, so that the surface of the 45 rug will present the appearance of a continuously extending pile surface and conceal the individual tufting and conceal the strand-like or bundled condition of the filaments at the base of each tuft where the strand penetrates the backing fabric.

It is necessary to bring the individual tufts into such close proximity to one another that the spreading of the free ends of the filaments will unite or intermesh the constituent filaments of proximate tufts into a continuous intermeshing surface in which the individual rayon filaments are free to catch and reflect light and produce the sheen-like effect above referred to.

After the rug has been stitched to form 55 tufts of the character mentioned, it still presents the effect of individual tufts, and in order to more completely separate the filaments and give to the rug the intended texture, it is necessary to either subject the rug to a dyeing or a washing treatment.

The invention in its most perfected form 60 contemplates the use of white or undyed thrown rayon strands which are preferably stitched through a white backing, and the 65 employment of undyed materials permits the rug to be dyed to the desired color after the tufting operation has been performed.

The extreme fineness and quality of the 70 thrown rayon filaments permits the rug, after 75 tufting, to be dyed by immersion for a few minutes in a suitable dye, during which limited period it has been found that the tips of the individual filaments, which are of gossamer fineness, will more quickly absorb the 80 dye and thus acquire a deeper shade of color than the underlying portions of the tufts, and it has also been found that the immersion in the dye liquid serves to more perfectly 85 spread or separate the filaments and intermesh them together to afford a continuous surface texture, so that, after removal from the dye liquid, and after drying, the rug will present an extremely soft, smooth and even fur-like texture, which effect is enhanced by 90 reason of the fact that the tips are more deeply colored, so that when the surface of the rug is stroked down, the underlying lighter colored portions of the rayon will be more or less exposed to give an effect very closely resembling that of natural fur.

If it is desired to further increase the luster of the rug, after dyeing, the same can be subjected to a bath of soluble oil, which completes the treatment and affords a rug

of extremely soft and fine texture and lustrous appearance.

Although it is preferred to tuft the rug with undyed strands of thrown rayon, a similar result may be attained by the use of dyed strands, which after tufting are subjected to washing in a soapy solution, which serves to spread and distend the individual rayon filaments in the manner previously referred to in connection with the dyeing operation. The rug in this instance also can be finished by the oil treatment previously mentioned.

In order to more completely disclose the details of the present invention, the various steps involved are illustrated in the accompanied drawing, wherein,—

Figure 1 illustrates a bundled and but slightly twisted strand of thrown rayon;

Fig. 2 illustrates the loops formed during the tufting operation and before the individual loops are cut to form tufts;

Fig. 3 illustrates the formation of the tufts after the loops have been severed; and

Fig. 4 illustrates the final condition of the rug after dyeing or washing to distend the filaments and obliterate the tufting effect.

In the drawing, the original thrown rayon strand A is stitched through the backing fabric B to form loops C, which are next cut to present the free ends D of the thrown rayon strand, which are afterwards spread or distended to present a substantially continuous pile surface E, as in Fig. 4.

Of course, it will be understood that the continuity of the pile surface will depend in considerable measure upon the closeness with which the tufts are spaced, and it will not always be possible to completely eliminate the effects of the tufting, so that in some cases, a slight ribbing effect will be observable in the completed rug, due to the formation of rows of stitching, but in all cases the tufting or stitching effect will be largely, if not entirely, concealed or obliterated, so that the completed rug will in a large measure present the appearance of natural fur.

Although I have referred to the product of the present invention as a rug, it will be understood that I do not limit such product strictly to use as a rug, but on the contrary intend to include in that designation any fabric having characteristic features of the present invention, whether used as a floor covering, or as an imitation fur intended for wearing apparel, or for any other purpose to which the present invention may be put.

It will also be understood that under the term "thrown rayon" I include a rayon strand of loosely bundled formation having filaments of gossamer-like fineness and having the capacity to separate or distend under the present treatment, but that I do not include strands of ordinary rayon of comparatively coarse texture and which are customarily tightly twisted together and do not have the

capacity for spreading or distension which is requisite in the manufacture of rugs having the characteristics of the present invention.

I claim:

1. The process of making rugs or the like, which consists in closely tufting a backing with loosely bundled strands of thrown rayon having filaments of gossamer-like fineness, and in thereafter subjecting the rug to a bath in a liquid dye to separate, distend and intermesh the free filament ends of the tufts to afford a substantially continuous and unbroken fur-like surface, and to dye the tips of the filaments to a deeper shade than the underlying portions of the tufts.

2. The process of making rugs or the like, which consists in closely tufting a backing with loosely bundled strands of thrown rayon having filaments of gossamer-like fineness, and in thereafter subjecting the rug to a bath in a liquid dye to separate, distend and intermesh the free filament ends of the tufts to afford a substantially continuous and unbroken fur-like surface, and to dye the tips of the filaments to a deeper shade than the underlying portions of the tufts, and in finally applying oil to the fur-like surface to increase the luster.

3. A rug or the like of the character described, including a backing having secured thereto closely spaced tufts, each tuft having its base portion in compacted relation and entered through the backing, and having its free tip ends distended to afford a substantially continuous fur-like surface, the tufts being formed of loosely bundled strands of thrown rayon composed of filaments of gossamer-like fineness, and the filaments of each tuft extending outwardly in diverging and progressively separated relation, and the marginal filaments of individual tufts contacting and intermeshing with the filaments of contiguous tufts to conceal the tufting arrangement, and the rug being dyed to impart a deeper coloration to the surface tips of the filaments than to the underlying portions thereof.

In witness that I claim the foregoing I have hereunto subscribed my name this 12th day of February, 1930.

PHILIP C. WAITE.

120

125

130